

## UNITED STATES PATENT OFFICE

2,131,719

METHOD OF IMPROVING THE SURFACE OF  
COPPER AND COPPER ALLOY CASTINGSCyril Stanley Smith, Cheshire, Conn., assignor to  
Anaconda Copper Mining Company, New York,  
N. Y., a corporation of MontanaNo Drawing. Application October 16, 1937,  
Serial No. 169,462

4 Claims. (Cl. 22—214)

It is customary in the production of ingots or castings of deoxidized copper or copper alloys to pour the molten metal into a metal mold dressed with some oily or carbonaceous materials. The exact manner in which the dressing acts is rather obscure but its function is to prevent the metal from sticking to the mold and so to give a clean smooth surface to the resulting casting. Through long years of trial and error casters have arrived at certain compositions, usually containing an oil and almost always some form of solid carbon which will give good results with a particular alloy, but in many cases it is still very difficult to obtain a casting with a really good surface. The bottom of the casting or other places where the stream of metal strikes against the mold is particularly apt to be bad, for the splashed drops of metal will frequently not melt into the main body and will remain, causing surface defects.

I have found that the introduction of a small amount of a volatile flux, such for example as ammonium chloride, into the bottom of a mold previously dressed in the usual way will considerably improve the surface of the bars and especially will benefit the extreme lowest part of the casting which is most liable to have surface defects if cast without any addition.

As a particular example of the application of my invention I have found that in casting a 350 pound bar of oxygen-free copper in a vertical copper mold dressed with a mixture of mold oil and graphite with or without an addition of bone black, the surface can be greatly improved by the introduction of about ten grams of powdered ammonium chloride in the bottom of the mold in such a location that the stream of metal on reaching the bottom strikes the ammonium chloride and so vaporizes it. This copper was melted in the presence of charcoal in a direct arc electric furnace and poured out of contact with air at a temperature of about 2150° F. at a rate of about 350 pounds per minute, but as described later I have found that these conditions may be varied.

It is well known that slow pouring gives sound bars when copper is cast in oil dressed molds but this usually results in a poor surface. Fast pouring improves the surface but frequently causes internal shrinkage cavities. The presence of ammonium chloride in the mold, according to my invention, produces a good surface on bars that have been poured at a slow enough rate to be sound. The ammonium chloride can be dropped in from the top of the mold, or it may be placed on the bottom plate before closing the mold, or it may be introduced in any other way. The amount

of ammonium chloride may vary from only a fraction of a gram up to several hundred grams depending on the size and particular conditions of casting and will vary with the type and shape of mold, and the temperature and rate at which the molten metal is poured, the height through which it falls and many other factors. The ammonium chloride should, however, always be at least partly vaporized or dissociated by contact with the hot metal.

Another way of introducing the ammonium chloride into the mold is by adding it to the dressing itself, and this can be done by mixing it as a dry powder in an oily dressing, or as an aqueous solution in those types of dressing consisting of a suspension of bone ash, bone black, and/or carbonaceous material in water, the dressing being allowed to dry on the surface of the mold. However, my experience shows it is preferable to place the dry ammonium chloride in the bottom of a previously dressed mold as above described.

When pouring deoxidized copper into oil dressed molds water is sometimes allowed to run in at the same time as the copper for the purpose of improving the surface. I have found that the use of an aqueous solution of ammonium chloride in place of water still further improves the surface. Additional ammonium chloride may also be placed in the bottom of the mold before casting is commenced either dry or in concentrated solution and will be effective when either water or ammonium chloride solution is introduced with the copper.

Additions of ammonium chloride in the mold may be advantageously employed not only in casting deoxidized or oxygen-free copper but also in the casting of copper alloys such as, for example, the brasses, bronzes, the silicon bronzes, copper nickel alloys and alloys of copper with aluminum or with cadmium. In each case the amount necessary and the exact method of application will vary, depending on casting conditions as outlined above. Ammonium chloride may also be used in sand molds for making castings of deoxidized copper or copper alloys. I have found that the addition of ammonium chloride is generally less effective in the casting of these copper alloys than in making castings of oxygen free or deoxidized copper.

I have also found that phosphorus pentoxide, phosphoric acid, and ammonium phosphate have a similar effect when placed on the bottom of the mold and the volatile metallic chlorides such as the chlorides of iron, aluminum, zinc, and cad-

mium are also effective. These substances have in common the property of volatility and the power of attacking metallic oxides which characterizes a flux. Although any of these volatile fluxes is effective in improving the surface of copper castings when introduced into the mold in substantially the same manner and amount as described above for ammonium chloride, in general I prefer to use ammonium chloride since it is effective, cheap, and is not deliquescent under ordinary atmospheric conditions.

Having thus set forth the nature of my invention, what I claim is:

1. The method of improving the surface of castings of copper and its alloys which comprises introducing a volatile flux into a dressed metallic mold and pouring the molten metal therein.

2. The method of improving the surface of castings of copper and its alloys which comprises introducing ammonium chloride into the mold and then pouring the molten metal therein.

3. The method of casting copper and its alloys which comprises pouring the molten metal into a mold containing a volatile metallic chloride.

4. The method of casting copper and its alloys which comprises dressing a metal mold with oily or dry carbonaceous material to prevent the copper sticking to the mold surfaces, placing in the mold cavity a quantity of ammonium chloride, and pouring the molten metal or alloy into the mold.

CYRIL STANLEY SMITH. 15